

## UNITED STATES PATENT OFFICE

2,095,400

METHOD FOR IMPROVING STEEL AND  
STEEL SHEETSCharles A. Scharschu, Brackenridge, Pa., assignor  
to Allegheny Steel Company, a corporation of  
PennsylvaniaNo Drawing. Application June 21, 1935,  
Serial No. 27,748

6 Claims. (Cl. 75—127)

My present invention relates to a process and an alloy compound for improving the properties of steel and steel sheets and more especially for eliminating seams from steel and off-color areas 5 from polished steel sheets. The present application is a continuation in part of an application filed by me on Dec. 19, 1931, under Ser. No. 582,177.

It is well-known that many stainless steel alloys 10 and articles of manufacture fabricated therefrom are today used for ornamental purposes. This use of stainless steel and stainless steel sheets has found wider and wider adaptation particularly in modern constructions both of domestic and of 15 commercial nature. For such purposes, it is apparent that the appearance of the steel and steel sheets must not only be attractive physically but must be uniform. Many such products have, however, been observed to exhibit defects which 20 either mar their appearance, limit their application or prohibit their use for ornamental purposes. In some cases, these defects have actually prevented the use of stainless steel products for some types of installations or have resulted in the 25 necessity for reworking the defective pieces to improve them. In other cases, the defects have caused relegation of these products to minor or inconspicuous locations. This necessarily results in an economic loss and at the same time increases the cost of acceptable stainless steel products 30 for ornamental purposes.

It has been observed that these defects are generally of two types. The type of defect exhibited by stainless steel, e. g., rounds, is known as a 35 seam and apparently consists of a relatively narrow imperfection, depression or trough which has comparatively little width and depth but which has considerable length which may amount, in some cases, to several inches, more or less. The type of defect exhibited by polished steel sheets is what is known as off-color areas. When these areas are present in the polished steel sheets spots or localized areas appear either 40 darker or lighter than the remainder of the sheet. Some of these off-color areas are darker than the 45 main body of the sheet when viewed at one angle and lighter than the main body of the sheet when viewed at another angle. As above pointed out, these defects limit the use of ornamental 50 stainless steel and cause perfect material to be increased in price.

It is believed by some that these off-color areas result from a scattering of light. If such is true there must be a physical defect in the material 55 which causes such light-dispersive or light-refractive phenomena. It is also thought that these defects result from the type of deoxidizer used during the production of the steel because when certain deoxidizers are used it is known 60 that the resulting steel contains a relatively large

number of inclusions and various other defects but that certain other deoxidizers produce steels exhibiting fewer defects. It is believed likely that the products of deoxidation find their way into the steel and constitute foreign matter with respect to their composition as compared to the steel. Metallurgists know that a small portion of all deoxidizers which are added to slags pass into the steel prior to effecting complete deoxidation of the steel. Inasmuch as deoxidizers are 10 invariably reducing in nature they exert a reducing effect upon metallic oxides present in the steel and frequently form non-metallic compounds which are either very difficult or even impossible to remove.

Where I refer to stainless steel or stainless steel sheets, especially polished steel and steel sheets, I mean in particular such products of the so-called 18-8 type which contain about 18% chromium, about 8% nickel, low carbon—usually 15 up to about .3%—low sonim content, and with the balance substantially all iron. I do not, however, exclude other types of stainless steel or iron but on the contrary I particularly mean to include all such which are adaptable for ornamental purposes.

I have discovered that stainless steel sheets and rounds made from stainless steel can be produced which are substantially entirely free from the above noted and other defects and the production of such forms one of the objects of this 20 invention.

Another object resides in adding to the slag during the production of the steel a certain alloy compound which results in the production of 25 sheets and rounds very substantially free from the noted defects.

Another object is to bring about a peculiar reducing action during the manufacture of the steel by adding to the slags used in the normal 30 refining of the steel an alloy compound of the nature hereinafter set forth.

A still further object is to produce stainless steel sheets and rounds of uniform high grade 35 adaptable for ornamental use by a modified steel-making process.

Other objects and advantages are to reduce the slags used during the normal manufacture of steel by means of an alloy compound composed primarily of calcium and silicon, together with 40 such other objects and advantages as will be understood by those versed in this art.

I am aware that finely divided silicon, e. g., as ferro-silicon, has heretofore been used to reduce the slag commonly used in making stainless steels 45 together with the fact that several other reducing or deoxidizing agents have been suggested or tried. My observations and experience have been, however, that steels made by known methods all produce material which is defective at 50

least to some extent and which, therefore, is not widely applicable to ornamentation. In particular, stainless steels made by known practice exhibit the foregoing defects, when polished or when turned down in a lathe, to a greater or lesser extent but to an extent sufficient to cause the rejection of an appreciable part of the steel for ornamental uses.

In contradistinction to the foregoing, I have discovered that if I add an alloy compound of calcium and silicon, as hereinafter more fully set forth, a highly improved steel results which is substantially entirely free from the seams and off-color areas mentioned above. My alloy compound containing calcium and silicon is added to the slags normally used in steel making operations. Such slags are frequently composed chiefly of lime and silica to which fluorspar has been added to render them more fluid. My calcium silicon alloy compound can be added to such a slag or to other slags as will be pointed out hereinafter.

I find that my alloy compound may, like more conventional deoxidizers, be added to the slag during the latter part of the deoxidation period. I prefer, however, to add the alloy compound to the slag at or near the beginning of the deoxidation period. Thus, the alloy compound is present and in contact with the slag throughout substantially the entire deoxidation period which produces somewhat better and more complete results than adding the alloy compound at or near the end of the deoxidation period.

In order that my present invention and the manner of carrying it out may be clear to those skilled in this art I have reproduced hereinbelow the pertinent data concerning what will be called heat No. 18,010. In accordance with the following table, I added the materials specified in the amounts set forth and at the times noted in the lefthand column.

#### Heat No. 18,010

| 45 | Time       | Remarks                                                                   | 45 |
|----|------------|---------------------------------------------------------------------------|----|
|    | 7:00 A. M. | Heat started                                                              |    |
|    | 4:23 P. M. | Slag removed                                                              |    |
| 50 | 4:25 P. M. | Added new slag containing 400# of lime and 105# of fluorspar              |    |
|    | 4:50 P. M. | Added 10# of calcium silicide and 10# of lime to the new slag             |    |
|    | 5:00 P. M. | Added 10# of calcium silicide and 10# of lime to the slag                 |    |
|    | 5:10 P. M. | Added 10# of calcium silicide and 10# of lime to the slag                 |    |
|    | 5:20 P. M. | Added 10# of calcium silicide and 20# of lime to the slag                 |    |
|    | 5:30 P. M. | Added 10# of calcium silicide and 10# of lime to the slag                 |    |
|    | 5:40 P. M. | Added 5# of calcium silicide, 5# of lime and 10# of fluorspar to the slag |    |
|    | 5:50 P. M. | Added 5# calcium silicide and 25# of lime to the slag                     |    |
| 55 | 6:00 P. M. | Added 10# of calcium silicide and 10# of lime to the slag                 | 50 |
|    | 6:10 P. M. | Added 10# of calcium silicide and 10# of lime to the slag                 |    |
|    | 6:20 P. M. | Added 10# of calcium silicide to the slag                                 |    |
|    | 8:15 P. M. | Alloying additions added:—                                                |    |
|    | 8:25 P. M. | Added 10# of calcium silicide and 10# of lime to the slag                 |    |
|    | 8:30 P. M. | Added 10# of calcium silicide and 10# of lime to the slag                 |    |
|    | 8:45 P. M. | Added 10# of calcium silicide and 10# of fluorspar to the slag            |    |
| 60 | 8:53 P. M. | Added 10# of calcium silicide and 10# of lime to the slag                 | 60 |

From the foregoing example it will be apparent that the slag and flux (lime and fluorspar) together constituted 675# and that the total additions of calcium silicide amounted to 140#. Thus, in this particular instance the weight of calcium silicide added amounted to approximately 20% of the weight of the slag and flux.

In the above example the calcium silicide utilized contained approximately 20 to 30% of calcium and about 80 to 70% of silicon although the exact proportions may be varied somewhat above or below these figures without departing from the spirit of the invention. I prefer to use the cal-

cium silicide in finely divided condition. This condition may be reached either by grinding calcium silicide to a finely divided condition or by preparing it, e. g., chemically by precipitation, directly in a finely divided condition as will be understood by those familiar with the handling of such materials. In its simplest form, my new alloy compound is substantially calcium silicide with or without minor percentages of extraneous but harmless materials and in such case may be closely enough indicated by the chemical notation CaSiZ.

I am not limited, however, to an alloy compound containing substantially only calcium and silicon. I contemplate the substitution or replacement of at least a part of the silicon content by other suitable metals such as manganese although I do not intend that manganese shall be the only replacement metal. Other metals may be used for replacement purposes instead of manganese where they have those properties and characteristics suitable for use in connection with the present invention. Silicon replacement may be proportionate to the atomic weights of the elements involved although I am not limited to only this type of replacement. Where the silicon is replaced in part or in whole by manganese or other elements, my alloy compound cannot be designated by a simple chemical formula since it is more likely to be a complex association of a number of chemical compounds as will be understood by those familiar with chemical reactions.

I have discovered, however, that the use of calcium silicide, or some modification or derivative thereof as above indicated, enables me to produce sheets and rounds which are substantially entirely free from the defects above described. I wish it to be understood that while I have indicated the addition of 140# of calcium silicide in the foregoing example I am not limited to such a figure. The precise or even approxi-

mate amount of calcium silicide or derivative which is to be used in any particular heat of steel must necessarily depend upon the severity, known or expected, of the defects likely to be exhibited by the particular analysis of steel being made. The amount of calcium silicide or derivative to be used can, however, be readily determined by a simple test or by trial and error. I employ enough calcium silicide to at least overcome the defects above mentioned and preferably I add a slight excess thereover since such an excess exerts no harmful effects upon the steel and ensures the elimination of all the defects.

While I have indicated above the probable modus operandi of the calcium silicide addition whether or not the theory involved is correct or not is immaterial, because calcium silicide used as herein explained produces the results stated and makes possible the accomplishment of the objects noted. Whether the use of calcium silicide according to my invention produces products of deoxidation of an unusual nature such that they diffuse from the steel to the slag or whether the calcium silicide in accordance with my invention results in some peculiar or unusual refinement of the steel in certain respects I am not positive, but, as already stated, the practice of my invention invariably produces the results sought.

As I have above stated my invention is not limited to the use of any particular slag and the example of lime and fluorspar has been given merely for exemplary purposes. I have found that since the slag is merely a vehicle for carrying out certain chemical and/or physical reactions which are necessary in the refining of steel my invention operates equally well with slags of other types or compositions. For instance, I have observed that if a slag composed of lime and alumina or lime and other suitable refractory oxides so proportioned as to give the desired fluidity are used in the manner known by those skilled in steel making, the objects of my invention are equally well accomplished in connection therewith and the advantages noted still exist. I, therefore, wish it to be understood that the composition of the slag is inconsequential insofar as my present invention is concerned, and I have found that in general it is not possible to lay down a general rule concerning the proportional relationship between the amount of calcium silicide or the like utilized and the weight of the slag and flux.

What I claim as new and desire to secure by Letters Patent is:

1. A process of making stainless steel free from seams and off-color areas which comprises preparing a suitable molten bath under a slag, removing the slag, forming a new slag thereon, and adding calcium silicide to the slag in sufficient amount to make it possible to produce stainless steel free from such seams and off-color areas, the calcium silicide being added in small increments at least some of which are accompanied by slag-forming additions.

2. A process of making stainless steel free from seams and off-color areas which comprises preparing a suitable molten bath under a slag, removing the slag, forming a new slag thereon, and adding calcium silicide to the slag in sufficient amount to make it possible to produce stainless steel free from such seams and off-color areas,

the calcium silicide being added in suitable increments and each such increment being added a relatively short period of time after the preceding increment, the calcium silicide additions being interrupted at a suitable time while the requisite alloying additions are made to the bath. 5

3. A process of making stainless steel free from seams and off-color areas which comprises preparing a suitable molten bath under a slag, removing the slag, forming a new slag thereon, 10 and adding calcium silicide to the slag in sufficient amount to make it possible to produce stainless steel free from such seams and off-color areas, and calcium silicide being added in small increments at least some of which are accompanied by 15 slag-forming additions, the calcium silicide and slag-forming additions being interrupted while the requisite alloying additions are made to the bath.

4. A method of making stainless steel products 20 adapted for ornamental uses and free from seams and off-color areas which comprises preparing a suitable molten bath under a slag, removing the slag and substituting a slag of lime and fluorspar, promptly beginning the addition of relatively 25 closely spaced increments of calcium silicide, at least some of which are accompanied by slag-forming materials, interrupting the additions to incorporate suitable alloying ingredients in the bath, and resuming the calcium silicide additions 30 until a predetermined total amount has been added.

5. A process of making ornamental 18-8 sheets and rounds substantially free from seams and off-color areas which comprises preparing a molten 35 bath of low carbon iron, removing the slag which forms thereon, adding materials including lime and fluorspar to form a new slag, periodically adding calcium silicide, lime and fluorspar to the new slag, interrupting the additions to make 40 alloying additions of chromium and nickel and delaying resumption of the other additions until the alloying additions are assimilated by the bath.

6. A process of making chromium nickel stainless steel sheets and rounds substantially entirely 45 free from seams and off-color areas which comprises making up a molten bath of iron, removing slag therefrom, adding materials including lime and fluorspar to form a new slag on the bath, incrementally adding calcium silicide and lime to 50 the slag, occasionally adding fluorspar to the slag for slag control, adding alloying agents and completing the additions of calcium silicide, lime and fluorspar, finishing the heat, forming it into ingots and manufacturing sheets and rounds from 55 such ingots.

CHARLES A. SCHARSCHU.